

## UNITED STATES PATENT OFFICE

2,131,195

## PRODUCTION OF DRYING OILS

Helmuth G. Schneider and Julius V. Sommer,  
Elizabeth, N. J., assignors to Standard Oil De-  
velopment Company, a corporation of Dela-  
ware

No Drawing. Application June 9, 1934,  
Serial No. 729,800

14 Claims. (Cl. 196—142)

This invention relates to the production of drying oils from hydrocarbons and especially from petroleum oils.

It is well known that vapor phase cracked 5 gasolines, especially gasolines produced by vapor phase cracking of high boiling mineral oils at a temperature of about 1100° F. and at a pressure of not over 150 pounds per square inch, are less stable on storage than ordinary cracking coil 10 distillates. It is believed that this is due to the presence of aromatic and unsaturated compounds, especially unsaturated compounds of the diole- fine series.

These vapor phase cracked gasolines are found 15 useful in preparing drying oils that are suitable for use in paints. Gasolines, produced by distillation of crude oils or by cracking high boiling point mineral oils at high pressures, are more stable and are not suitable for the production of drying 20 oils.

An object of this invention is to treat unsaturated hydrocarbon compounds to produce drying oils for use in paints. This and other objects of the invention will be understood from 25 the following description.

According to this invention, vapor phase cracked gasolines boiling up to 300° C. are preferentially oxidized, separated preferably by means of vacuum distillation, and polymerized. 30 The oxidation of the diolefines takes place more readily than ordinary olefines and the mechanism of the oxidation does not appear to be the same for the two types of unsaturated compounds. In many respects the oxidation of the diolefines 35 resembles the drying of linseed oil. Therefore, the diolefines are readily oxidized in the presence of saturated and unsaturated compounds and the oxidized diolefines are separated by means of distillation. The oxidation is generally carried 40 out in the liquid phase and at a temperature of about 50° to 150° C. and under superatmospheric pressures. For example, partial oxidation at 100° C. and 110 pounds pressure per square inch of vapor phase distillate with subsequent removal 45 of the lighter unoxidized material by distillation yields a heavy oil which dries to a non-tacky film when exposed to the air. This drying oil resembles linseed oil in that: (a) it absorbs oxygen from the air during the drying; (b) it gradually increases in viscosity on being kept at about 150° C.; (c) it dries more rapidly after being "boiled"; (d) driers such as cobalt, lead, copper, and manganese oleates greatly increase 50 the rate of oxidation and decrease the drying 55

time when the oil is exposed in thin films. The film formed on drying does not finger mark.

It has also been found that certain fractions of vapor phase cracked gasoline yield better drying oils than others. Fractions boiling between 40° C. and 108° C. and between 130° C. and 145° C. give the largest yields. Another factor that affects the yields is the amount of oxygen absorbed which varies as to the particular distillate used. However, large amounts of air or oxygen should be avoided since the quality of the drying oil drops off in proportion and a point is reached where the oxidized product no longer dries to a solid film as can be seen below.

Vapor phase gasolines, obtained by cracking at substantially atmospheric pressure, contain about 11% of diolefines and yield about 5% of drying oils under normal operating conditions. However, by polymerizing at 230° C. and under approximately 1,000 to 1,500 pounds per square inch pressure of nitrogen containing a very small percentage of air such as enough to make the oxygen content about 5%, the yield of drying oil was raised to 6-11% and the resulting oil, on drying, 15 20 25 formed a hard film.

In order to obtain a colorless drying oil, it has been found necessary to first treat the gasoline to remove any sulfur compounds that may be 30 present. This is generally done by refluxing the gasoline with metallic sodium, copper oxide or lead oxide.

The following example illustrates the effect 35 of time of oxidation on the yield and quality of the drying oil:

| Time of oxidation | Yield of drying oil | Drying time for pressure drop of 250 mm.* |             | 40  |
|-------------------|---------------------|-------------------------------------------|-------------|-----|
|                   |                     | Without drier                             | With drier  |     |
| 3½ hrs.....       | Percent<br>4.2      | Hours<br>160                              | Hours<br>46 | 46  |
| 7 hrs.....        | 6.8                 | (t)                                       | 137         | 137 |
| 11 hrs.....       | 7.0                 | (t)                                       | 180         | 180 |
| 15 hrs.....       | 8.5                 | (t)                                       | (t)         | 45  |

\* To compare the drying properties of oils, the rate of oxygen absorption is given as the time in hours required for a pressure drop of 250 mm. of mercury in a closed system containing known volumes of the respective oils attached to a manometer containing oxygen.

† Did not give the required pressure drop in 200 hrs.

The following table gives results of tests of three drying oils, described below, which illustrate the rate of oxygen absorption of the drying 50 55

oils of the present invention, as compared with linseed oil:—

| 5  | Time of contact of oil and oxygen | Linseed oil | Oil "A"   | Oil "B"   | Oil "C"   |
|----|-----------------------------------|-------------|-----------|-----------|-----------|
| 10 | 70                                | Mm.<br>10   | Mm.<br>20 | Mm.<br>30 | Mm.<br>60 |
|    | 100                               | 30          | 50        | 62        | 110       |
| 15 | 140                               | 55          | 70        | 118       | 200       |

The figures are given as the rate of decrease of oxygen pressure in a closed system containing known volumes of the respective oil attached to a manometer. Oil "A" represents a drying oil obtained from a Mid-Continent gasoline boiling between 90° C. and 170° C. and produced by vapor phase cracking. Oil "B" represents a drying oil obtained from a gasoline produced by so-called gyro-process vapor phase cracking without pressure. Oil "C" represents a drying oil obtained from a gasoline boiling between 90° and 200° C. and produced by the DeFlorz process vapor phase cracking of a Mid-Continent oil.

It has been found that while the drying oils produced by oxidation of vapor phase gasoline at about 100° C. and 110 pounds air pressure possess many of the characteristics of linseed oil, the film produced on drying was too soft as it could be scratched with a finger nail. It has been found that a drying oil that dries to a harder film can be produced (1) by taking the oxidized drying oil produced by contacting with oxygen at 100° C. and 110 pounds air pressure for about 3½ hours, and treating the oil further by polymerization with nitrogen at more elevated temperatures and pressures, such as about 230° C. and 1500 lbs. per sq. in. for 17 hours.

(2) By oxidation of the gasoline with air (or an inert gas containing about 10 to 50% of oxygen) at more elevated temperatures and pressures such as about 230° C. and 1500 lbs. per sq. in. for 17½ hours so as to speed up the rate of initial polymerization during the formation of the oil, or

(3) By polymerizing the diolefines and gasoline at high pressures and in the presence of traces of oxygen such as 0.01 to 2.0% at about 230° C. for about 17 hours.

Larger amounts of the drying oil are produced by oxidation and polymerization at more elevated temperatures and pressures. A drying oil can be prepared from vapor phase cracked gasoline which, on exposure to air, dries to a hard film. The preferred temperatures and pressures for the production of drying oils from vapor phase gasoline are approximately 200° C. and 1000 to 1500 pounds per square inch respectively.

The following example illustrates the effects on a drying oil of the addition of 0.2% of a drier, such as cobalt oleate, on the drying rate. The rate of oxidation is given as the time required for a pressure drop of 250 mm.

| 65 | Oil "A" | Hours | Oil "B" | Hours |
|----|---------|-------|---------|-------|
|    | Oil "B" | 130   | Oil "C" | 26    |
| 70 | Oil "C" | 125   |         | 28    |
|    |         | 160   |         | 41    |

The oils used were obtained by oxidation of the diolefin, separated and polymerized.

In the appended claims the term "oxygen" is intended to mean free molecular oxygen substantially free from any ozone.

Having thus described the invention, it is not intended that it be limited by any of the specific examples given but it is desired to claim all inherent novelty as broadly as the prior art permits.

We claim:

1. A process for producing a drying oil which comprises subjecting a fraction of gasoline normally boiling between the approximate limits of 40° and 108° C. and obtained by vapor phase cracking of higher boiling mineral oils at a pressure of not over about 150 lbs. per square inch, in liquid phase to the action of a gas containing oxygen at a temperature between the approximate limits of 50° and 150° C. and at a pressure of about 100 lbs. per square inch, and recovering a drying oil from the product by distillation.

2. A process for producing a drying oil which comprises subjecting a fraction of gasoline obtained by vapor phase cracking of higher boiling mineral oils, in liquid phase to the action of a gas containing oxygen at a pressure substantially above atmospheric and at a temperature of about 50° to 230° C., recovering a drying oil from the product by distillation and polymerizing said drying oil at elevated temperature and pressure.

3. Process according to claim 2 in which the final polymerization step is carried out at a temperature of about 200° C. and at a pressure of about 1000 lbs. per square inch.

4. A process for producing oxidized hydrocarbons, which comprises subjecting in the liquid phase to the action of a gas containing oxygen at a pressure substantially above atmospheric and at a temperature of about 50° to 230° C., a narrow cut gasoline fraction having a boiling range spread of not over about 70° C. and capable of yielding superior oxidized hydrocarbons than a gasoline derived from the same crude petroleum but having the usual wide boiling range, said fraction to be treated with oxygen having been obtained by vapor phase cracking of higher boiling mineral oils.

5. Process according to claim 4 carried out at a temperature below about 150° C.

6. Process according to claim 4 carried out at a temperature between the approximate limits of 50 and 150° C. and at a pressure above about 100 pounds per square inch.

7. Process according to claim 4 carried out at a temperature above about 200° C. and at a pressure above about 1000 pounds per square inch.

8. Process according to claim 4 carried out at a temperature above about 200° C. and at a pressure above about 1000 pounds per square inch, using a gas containing not more than about 5% oxygen.

9. Process according to claim 4 in which the gasoline fraction treated is subjected to a preliminary sulfur removal treatment in order to produce a substantially colorless finished drying oil.

10. Process according to claim 4 in which a gasoline fraction normally boiling between the approximate limits of 40° and 108° C. is treated.

11. Process according to claim 4 in which a gasoline fraction normally boiling between the approximate limits of 130° and 145° C. is treated.

12. A process for producing a drying oil, which comprises subjecting in liquid phase to the action of a gas containing oxygen, at a pressure substantially above atmospheric and at a temperature of about 50 to 230° C. and for a time

adapted to produce optimum drying oil properties, a narrow cut gasoline fraction having a boiling range spread of not over about 70° C. and capable of yielding superior drying oils than the whole gasoline of the usual wide boiling range, and recovering a drying oil from the product by distillation.

13. A process for producing oxidized hydrocarbons, which comprises subjecting a fraction of gasoline obtained by vapor phase cracking of

higher boiling mineral oils, in liquid phase to the action of a gas containing oxygen, at a temperature between the approximate limits of 200 and 230° C. and a pressure above about 1000 pounds per square inch.

14. Process according to claim 13 in which an oxidizing gas is used containing not more than about 5% of oxygen.

HELMUTH G. SCHNEIDER.

JULIUS V. SOMMER.

5

10